



US010889779B2

(12) **United States Patent**  
**Aoyama**

(10) **Patent No.:** **US 10,889,779 B2**  
(b4) **Date of Patent:** **Jan. 12, 2021**

(54) **TRANSMISSION LUBRICATING OIL COMPOSITION**

(71) Applicant: **IDEMITSU KOSAN CO., LTD.**,  
Chiyoda-ku (JP)

(72) Inventor: **Kayoko Aoyama**, Sapporo (JP)

(73) Assignee: **IDEMITSU KOSAN CO., LTD.**,  
Chiyoda-ku (JP)

(\*) Notice: Subject to any disclaimer, the term of this patent is extended or adjusted under 35 U.S.C. 154(b) by 0 days.

(21) Appl. No.: **15/561,301**

(22) PCT Filed: **Jan. 25, 2016**

(86) PCT No.: **PCT/JP2016/051992**

§ 371 (c)(1),  
(2) Date: **Sep. 25, 2017**

(87) PCT Pub. No.: **WO2016/157960**

PCT Pub. Date: **Oct. 6, 2016**

(65) **Prior Publication Data**

US 2018/0100119 A1 Apr. 12, 2018

(30) **Foreign Application Priority Data**

Mar. 31, 2015 (JP) ..... 2015-074419

(51) **Int. Cl.**

**C10M 169/04** (2006.01)  
**C10M 145/14** (2006.01)  
**C10M 149/18** (2006.01)  
**C10M 157/04** (2006.01)  
**C10M 161/00** (2006.01)  
**C10M 129/74** (2006.01)  
**C10M 101/00** (2006.01)  
**C10M 107/02** (2006.01)  
**C10N 20/02** (2006.01)  
**C10N 20/04** (2006.01)  
**C10N 30/00** (2006.01)  
**C10N 30/02** (2006.01)  
**C10N 30/06** (2006.01)  
**C10N 40/04** (2006.01)  
**C10N 40/08** (2006.01)  
**C10N 40/16** (2006.01)  
**C10M 129/76** (2006.01)

(52) **U.S. Cl.**

CPC ..... **C10M 169/044** (2013.01); **C10M 101/00** (2013.01); **C10M 129/74** (2013.01); **C10M 145/14** (2013.01); **C10M 149/18** (2013.01); **C10M 157/04** (2013.01); **C10M 161/00** (2013.01); **C10M 169/04** (2013.01); **C10M 107/02** (2013.01); **C10M 129/76** (2013.01); **C10M 2203/003** (2013.01); **C10M 2203/1006** (2013.01); **C10M 2205/0285** (2013.01); **C10M 2207/283** (2013.01); **C10M 2207/287** (2013.01); **C10M 2207/288** (2013.01); **C10M 2207/289**

(2013.01); **C10M 2209/084** (2013.01); **C10M 2217/044** (2013.01); **C10N 2020/02** (2013.01); **C10N 2020/04** (2013.01); **C10N 2030/00** (2013.01); **C10N 2030/02** (2013.01); **C10N 2030/06** (2013.01); **C10N 2030/60** (2020.05); **C10N 2030/68** (2020.05); **C10N 2040/04** (2013.01); **C10N 2040/08** (2013.01); **C10N 2040/16** (2013.01)

(58) **Field of Classification Search**

CPC ..... C10N 2240/042; C10N 2240/044; C10N 2240/045; C10M 2205/003; C10M 2207/287; C10M 2207/288  
USPC ..... 508/591, 551, 554  
See application file for complete search history.

(56) **References Cited**

U.S. PATENT DOCUMENTS

4,280,916 A \* 7/1981 Richards ..... C10M 133/16 508/287  
4,537,696 A \* 8/1985 Beimesch ..... C10M 169/044 252/75  
4,686,055 A \* 8/1987 Horodysky ..... C10L 1/224 508/287  
5,137,980 A 8/1992 Degonia et al.  
5,395,539 A \* 3/1995 Chandler ..... C10M 133/16 252/77

(Continued)

FOREIGN PATENT DOCUMENTS

CN 101058761 A 10/2007  
CN 101300330 A 11/2008  
(Continued)

OTHER PUBLICATIONS

International Search Report dated Feb. 23, 2016, in PCT/JP2016/051992, filed Jan. 25, 2016.

(Continued)

*Primary Examiner* — Ellen M McAvoy

(74) *Attorney, Agent, or Firm* — Oblon, McClelland, Maier & Neustadt, L.L.P.

(57) **ABSTRACT**

Provided is a lubricating oil composition for a transmission having excellent gear properties, clutch properties, cooling properties, and electric insulating properties. The lubricating oil composition for a transmission preparing by blending (A) a base oil, (B) a viscosity index improver having a mass average molecular weight of 10,000 to 50,000, and (C-1) a polyamide and/or (C-2) a polyol ester, the base oil (A) including (A-1) a synthetic oil having a kinematic viscosity at 100° C. of 1.0 to 10.0 mm<sup>2</sup>/s.



## 1

TRANSMISSION LUBRICATING OIL  
COMPOSITION

## TECHNICAL FIELD

The present invention relates to a lubricating oil composition for a transmission.

## BACKGROUND ART

Hitherto, a lubricating oil composition for a transmission has been required to have gear properties and clutch properties.

The gear properties indicate, for example, seizure resistance or shear stability under a high load. In addition, the clutch properties indicate, for example, suppression of shift shock generated when a coefficient of friction increases at the time of clutch connection.

In addition, in recent years, with the spread of hybrid vehicles or electric cars, a lubricating oil composition for motor cooling is used, too. Since there is a case where such a lubricating oil composition comes into direct contact with a motor and cools it, or the like, the lubricating oil composition is required to have high insulating properties together with cooling properties.

In addition, in recent years, it is also required to make a lubricating oil composition have a combination of plural applications. For example, there is exemplified a case where by providing a lubricating oil composition for a transmission with cooling properties and insulating properties, the lubricating oil composition is made to have a combined use for a transmission and motor cooling.

As general lubricating oil compositions for a transmission, technologies of PTLs. 1 to 3 are proposed.

## CITATION LIST

## Patent Literature

PTL 1: JP 2-46635 A

PTL 2: JP 2008-208221 A

PTL 3: JP 2011-168677 A

## DISCLOSURE OF INVENTION

## Technical Problem

PTL 1 proposes a lubricating oil composition for a wet clutch or a wet brake containing a specified phosphoric acid ester amine salt and a specified fatty acid ester. The lubricating oil composition of PTL 1 is one realizing performances, such as good friction properties, thermal oxidative stability, corrosion resistance, rust preventing properties, etc.

PTL 2 proposes a lubricating oil composition for an automobile transmission containing an ethylene-propylene copolymer having a specified viscosity in a base oil having a specified viscosity. The lubricating oil composition of PTL 2 is one realizing a low viscosity as well as an excellent fatigue life.

PTL 3 proposes a lubricating oil composition for a continuously variable transmission containing a poly- $\alpha$ -olefin having specified properties and a polymethacrylate having a specified mass average molecular weight. The lubricating oil composition of PTL 3 is one realizing a low viscosity, a high viscosity index, a stable shear stability, and a long fatigue life.

## 2

However, all of the lubricating oil compositions of PTLs 1 to 3 could not be simultaneously satisfied with gear properties, clutch properties, cooling properties, and electric insulating properties.

5 An object of the present invention is to provide a lubricating oil composition for a transmission having excellent gear properties, clutch properties, cooling properties, and electric insulating properties.

## 10 Solution to Problem

In order to solve the aforementioned problem, the present invention provides a lubricating oil composition for a transmission, which preparing by blending (A) a base oil, (B) a viscosity index improver having a mass average molecular weight of 10,000 to 50,000, and (C-1) a polyamide and/or (C-2) a polyol ester, the base oil (A) including (A-1) a synthetic oil having a kinematic viscosity at 100°C. of 1.0 to 10.0 mm<sup>2</sup>/s.

## 20 Advantageous Effects of Invention

25 The lubricating oil composition for a transmission of the present invention is able to simultaneously satisfy gear properties (e.g., seizure resistance or shear stability under a high load), clutch properties (e.g., suppression of shift shock at the time of clutch connection), cooling properties, and electric insulating properties.

## 30 DESCRIPTION OF EMBODIMENTS

An embodiment of the present invention (hereinafter also referred to as "present embodiment") is hereunder described.

35 The lubricating oil composition for a transmission of the present embodiment is one preparing by blending (A) a base oil, (B) a viscosity index improver having a mass average molecular weight of 10,000 to 50,000, and (C-1) a polyamide and/or (C-2) a polyol ester, the base oil (A) including (A-1) a synthetic oil having a kinematic viscosity at 100°C. of 1.0 to 10.0 mm<sup>2</sup>/s.

In the present embodiment, the composition prescribed as the "composition preparing by blending the component (A), the component (B), and the component (C-1) and/or the component (C-2)" includes not only a "composition including the component (A), the component (B), and the component (C-1) and/or the component (C-2)" but also a "composition including a modified product resulting from modification of at least one component of the component (A), the component (B), and the component (C-1) and/or the component (C-2) in place of the foregoing component" or a "composition including a reaction product resulting from reaction of the component (A), the component (B), and the component (C-1) and/or the component (C-2)".

## 55 &lt;(A) Base Oil&gt;

The lubricating oil composition for a transmission of the present embodiment is one including a base oil as the component (A) blended therein. Examples of the base oil as the component (A) include a mineral oil and a synthetic oil.

60 In the present embodiment, it is required to include (A-1) a synthetic oil having a kinematic viscosity at 100°C. of 1.0 to 10.0 mm<sup>2</sup>/s as the component (A).

In the case where the component (A-1) is not included as the base oil as the component (A), the shear stability is lowered, so that the gear properties cannot be made excellent, and furthermore, the shift shock at the time of clutch connection is generated, so that the clutch properties cannot

be made excellent. In addition, in the case where the component (A-1) is not included, the cooling properties are insufficient, so that an increase of the viscosity in a low-temperature environment cannot be suppressed. On the other hand, when the component (A-1) is included as the base oil as the component (A), the gear properties and the clutch properties can be made excellent. Furthermore, when the component (A-1) is included, not only the cooling properties can be made excellent, but also the increase of the viscosity in a low-temperature environment can be suppressed.

In order to make it easy to exhibit an effect based on the aforementioned component (A-1), in the synthetic oil as the component (A-1), it is preferred that a kinematic viscosity at 100° C. and a kinematic viscosity at 40° C. fall within the following ranges, respectively.

The kinematic viscosity at 100° C. is preferably 1.1 to 5.0 mm<sup>2</sup>/s, and more preferably 1.2 to 2.5 mm<sup>2</sup>/s. The kinematic viscosity at 40° C. is preferably 2.0 to 20.0 mm<sup>2</sup>/s, more preferably 3.0 to 10.0 mm<sup>2</sup>/s, and still more preferably 4.0 to 6.0 mm<sup>2</sup>/s.

In the present embodiment, the kinematic viscosity and the viscosity index are those as measured in conformity with JIS K2283:2000.

Examples of the synthetic oil as the component (A-1) include a poly- $\alpha$ -olefin, such as polybutene, polyisobutylene, a 1-octene oligomer, a 1-decene oligomer, an ethylene-propylene copolymer, etc., a hydrogenated product of a poly- $\alpha$ -olefin, a polyphenyl ether, an alkylbenzene, an alkylnaphthalene, an ester oil, a glycol-based or polyolefin-based synthetic oil, and the like. Among those, from the viewpoint of making the gear properties excellent, a poly- $\alpha$ -olefin and/or a hydrogenated product of a poly- $\alpha$ -olefin is suitable.

The  $\alpha$ -olefin serving as a raw material of the poly- $\alpha$ -olefin may be either linear or branched.

The  $\alpha$ -olefin serving as a raw material of the poly- $\alpha$ -olefin has preferably 8 to 20 carbon atoms, and more preferably 8 to 12 carbon atoms. Among those, 1-decene having 10 carbon atoms is suitable.

The blending amount of the component (A-1) is preferably 1.0 to 10.0% by mass, more preferably 1.5 to 7.0% by mass, and still more preferably 2.0 to 5.0% by mass on the basis of the total amount of the lubricating oil composition for a transmission. When the blending amount of the component (A-1) is 1.0% by mass or more, the gear properties, the clutch properties, and the cooling properties can be made excellent; and when it is 10.0% by mass or less, deterioration of the gear properties to be caused due to an excessive reduction of the viscosity can be suppressed.

In addition, the blending amount of the component (A-1) is preferably 1.5 to 12.0% by mass, more preferably 2.0 to 10.0% by mass, and still more preferably 2.5 to 5.0% by mass on the basis of the total amount of the component (A).

The lubricating oil composition for a transmission of the present embodiment may include a base oil other than the component (A-1) as the base oil as the component (A).

As such a base oil, a mineral oil, or a synthetic oil whose kinematic viscosity at 100° C. falls outside the range of 1.0 to 10.0 mm<sup>2</sup>/s, is exemplified.

Examples of the mineral oil include a paraffin-based mineral oil, an intermediate mineral oil, and a naphthene-based mineral oil, each of which is obtained through a usual refining method, such as solvent refining, hydrogenation refining, etc., and the like; a wax isomerized oil which is produced through isomerization of a wax, such as a wax produced by the Fischer-Tropsch process (gas-to-liquid wax), a metal oil-based wax, etc.; and the like.

The mineral oil is preferably one having a kinematic viscosity at 40° C. in the range of 5 to 50 mm<sup>2</sup>/s and a kinematic viscosity at 100° C. in the range of 1.5 to 6 mm<sup>2</sup>/s.

The blending amount of the mineral oil is preferably 60.0 to 90.0% by mass, more preferably 60.0 to 80.0% by mass, and still more preferably 65.0 to 75.0% by mass on the basis of the total amount of the lubricating oil composition for a transmission.

The blending amount of the base oil as the component (A) is preferably 70 to 98% by mass, more preferably 70 to 90% by mass, and still more preferably 75 to 85% by mass on the basis of the total amount of the lubricating oil composition for a transmission.

<(B) Viscosity Index Improver>

15 The lubricating oil composition for a transmission of the present embodiment is one including (B) a viscosity index improver, a mass average molecular weight (Mw) of which is 10,000 to 50,000, blended therein.

According to a viscosity index improver having a mass 20 average molecular weight of less than 10,000, the viscosity index of the lubricating oil composition cannot be sufficiently improved, so that the effects of gear properties, clutch properties, and insulating effects are hardly stably exhibited in a wide temperature region. In addition, according to a viscosity index improver having a mass average molecular weight of more than 50,000, the shear stability is lowered, so that the gear properties cannot be satisfied.

On the other hand, when the viscosity index improver (B) having a mass average molecular weight (Mw) of 10,000 to 30 50,000 is blended in the lubricating oil composition for a transmission, the effects of gear properties, clutch properties, and insulating effects can be readily stably exhibited in a wide temperature region. In addition, when the viscosity index improver having a mass average molecular weight of 35 50,000 or less is used, an increase of the viscosity in a low-temperature environment can be suppressed.

The mass average molecular weight (Mw) of the viscosity index improver as the component (B) is preferably 15,000 to 45,000, and more preferably 20,000 to 40,000.

40 In the present embodiment, the "mass average molecular weight" refers to a molecular weight as expressed in terms of polystyrene by means of the gel permeation chromatography (GPC) measurement.

Examples of the viscosity index improver as the component (B) include an olefin-based polymer, such as an ethylene-propylene copolymer, etc., a styrene-based polymer, such as a styrene-diene hydrogenated copolymer, etc., a poly(meth)acrylate, and the like. Among those, a poly(meth)acrylate is suitable.

45 The monomer that constitutes the poly(meth)acrylate is an alkyl (meth)acrylate, and preferably an alkyl (meth)acrylate having a linear alkyl group having 1 to 18 carbon atoms or a branched alkyl group having 3 to 34 carbon atoms.

Preferred examples of the monomer that constitutes the 50 alkyl (meth)acrylate include methyl (meth)acrylate, ethyl (meth)acrylate, propyl (meth)acrylate, butyl (meth)acrylate, pentyl (meth)acrylate, hexyl (meth)acrylate, heptyl (meth)acrylate, heptyl (meth)acrylate, octyl (meth)acrylate, nonyl (meth)acrylate, decyl (meth)acrylate, dodecyl (meth)acrylate, tetra (meth)acrylate, hexa (meth)acrylate, octadecyl (meth)acrylate, and the like. Copolymers using two or more of these monomers may also be used. The alkyl group of such a monomer may be either linear or branched.

55 In addition, examples of the alkyl (meth)acrylate having a branched alkyl group having 3 to 34 carbon atoms include isopropyl (meth)acrylate, 2-ethylhexyl (meth)acrylate, 3,5, 60 5-trimethylhexyl (meth)acrylate, 2-butyloctyl (meth)acry-

late, 2-hexyldecyl (meth)acrylate, 2-octyldodecyl (meth)acrylate, 2-decytetradecyl (meth)acrylate, 2-dodecylhexadecyl (meth)acrylate, and 2-tetradecyloctadecyl (meth)acrylate.

The blending amount of the viscosity index improver as the component (B) is preferably 1.0 to 20.0% by mass, more preferably 3.0 to 15.0% by mass, and still more preferably 5.0 to 10.0% by mass on the basis of the total amount of the lubricating oil composition for a transmission. When the blending amount of the component (B-1) is 1.0% by mass or more, the aforementioned effects based on the component (B) can be readily obtained, and when it is 20.0% by mass or less, an increase of the viscosity can be suppressed.

It is preferred that the lubricating oil composition for a transmission of the present embodiment does not contain a viscosity index improver having a mass average molecular weight of less than 10,000 and/or a viscosity index improver having a mass average molecular weight of more than 50,000.

<(C-1) Polyamide and (C-2) Polyol Ester>

The lubricating oil composition for a transmission of the present embodiment is one including (C-1) a polyamide and/or (C-2) a polyol ester blended therein.

In the case where the polyamide (C-1) and/or the polyol ester (C-2) is not blended in the lubricating oil composition for a transmission, the shift shock is generated at the time of clutch connection, so that the clutch properties cannot be made excellent. On the other hand, by blending the polyamide (C-1) and/or the polyol ester (C-2) in the lubricating oil composition for a transmission, the clutch properties can be made excellent.

In the lubricating oil composition for a transmission of the present embodiment, though at least one of the polyamide (C-1) and the polyol ester (C-2) has only to be blended, in the case where both of the polyamide (C-1) and the polyol ester (C-2) are blended, such is suitable from the standpoint that the clutch properties can be made more excellent.

Examples of the polyamide as the component (C-1) include amide compounds obtained through reaction between an amine compound and a carboxylic acid compound.

Examples of the amine compound that constitutes the polyamide (C-1) include aliphatic polyamines.

In the aliphatic polyamine, its total carbon number is preferably 6 to 30, more preferably 12 to 24, and still more preferably 16 to 20.

Specific examples of the aliphatic polyamine include hexamethylenediamine, 1,7-diaminoheptane, 1,8-diaminoctane, 1,9-diaminononane, 1,10-diaminodecane, 1,11-diaminoundecane, 1,12-diaminododecane, 1,13-diaminotri-decane, 1,14-diaminotetradecane, 1,15-diaminopentadecane, 1,16-diaminohexadecane, 1,17-diaminoheptadecane, 1,18-diaminoctadecane, 1,19-diaminononadecane, 1,20-diaminoeicosane, 1,21-diaminoheneicosane, 1,22-diaminodocosane, 1,23-diaminotricosane, 1,24-diaminotetacosane, 1,25-diaminopentacosane, 1,26-diaminohexacosane, 1,27-diaminoheptacosane, 1,28-diaminoctacosane, 1,29-diaminononacosane, 1,30-diaminotriacontane, hexenyl diamine, heptenyl diamine, octenyl diamine, nonenyl diamine, decenyl diamine, undecenyl diamine, dodecenyl diamine, tridecenyl diamine, tetradecenyl diamine, pentadecenyl diamine, hexadecenyl diamine, heptadecenyl diamine, octadecenyl diamine, nonadecenyl diamine, eicosenyl diamine, heneicosenyl diamine, docosenyl diamine, tricosenyl diamine, tetracosenyl diamine, pentacosenyl diamine, hexacosenyl diamine,

heptacosenyl diamine, octacosenyl diamine, nonacosenyl diamine, triacontenyl diamine, triethylenetetramine, tetraethylenepentamine, pentaethylenhexamine, di(methylethylene)triamine, dibutylenetriamine, tributylene tetramine, pentapentylene hexamine, tris(2-aminoethyl)amine, and the like.

In the carboxylic acid compound that constitutes the polyamide (C-1), the carbon number of the hydrocarbon group is preferably 6 to 30, more preferably 8 to 24, still more preferably 12 to 24, and yet still more preferably 18 to 22.

In addition, the carboxylic acid compound that constitutes the polyamide (C-1) is preferably a monovalent fatty acid. The foregoing fatty acid may be either linear or branched, and may be either saturated or unsaturated.

Examples of such a carboxylic acid compound include saturated fatty acids, such as caproic acid, enanthic acid, caprylic acid, 2-ethylhexanoic acid, pelargonic acid, capric acid, lauric acid, myristic acid, palmitic acid, margaric acid, stearic acid, isostearic acid, arachidic acid, behenic acid, lignoceric acid, etc.; and unsaturated fatty acids, such as lauric acid, myristoleic acid, palmitoleic acid, oleic acid, linoleic acid, erucic acid, etc.

From the viewpoint of making the clutch properties excellent, the polyamide as the component (C-1) preferably has a molecular weight of 1,000 or less.

Examples of the polyol ester as the component (C-2) include esters obtained through reaction between a polyol and a carboxylic acid compound.

In addition, though the polyol ester as the component (C-2) may be either a fully esterified compound or a partial ester, from the viewpoint of making the clutch properties excellent, a partial ester is preferred.

The polyol that constitutes the polyol ester (C-2) is preferably an aliphatic polyol having 2 to 15 carbon atoms, and more preferably an aliphatic polyol having 2 to 8 carbon atoms.

Specific examples of the polyol include ethylene glycol, propylene glycol, butylene glycol, neopentyl glycol, trimethylolpropane, trimethylolpropane, ditrimethylolpropane, glycerin, pentaerythritol, dipentaerythritol, tripentaerythritol, sorbitol, and the like. Among those, from the viewpoint of making the clutch properties excellent, trivalent or multivalent aliphatic polyols are suitable, and above all, glycerin is suitable.

As the carboxylic acid compound that constitutes the polyol ester (C-2), it is preferred to use a fatty acid having 12 to 24 carbon atoms. The fatty acid as referred to herein may be either linear or branched, and saturated and unsaturated alkyl groups are included.

In addition, the carboxylic acid compound may be a monovalent carboxylic acid, such as stearic acid, oleic acid, etc., and may also be a polyvalent carboxylic acid, such as succinic acid, adipic acid, pimelic acid, azelaic acid, sebacic acid, phthalic acid, isophthalic acid, etc.

Among these carboxylic acid compounds, stearic acid and oleic acid are suitable.

A total blending amount of the component (C-1) and the component (C-2) is preferably 0.01 to 5.0% by mass, more preferably 0.02 to 2.5% by mass, and still more preferably 0.05 to 1.0% by mass on the basis of the total amount of the composition. When the total blending amount of the component (C-1) and the component (C-2) is 0.01% by mass or more, the clutch properties can be made excellent, and when it is 5.0% by mass or less, a reduction of the clutch capacity can be suppressed.

## &lt;Additives&gt;

The lubricating oil composition for a transmission of the present embodiment may contain additives, such as a friction modifier, an antioxidant, a dispersant, a pour-point depressant, an antifoaming agent, etc.

The blending amount of the additive is preferably 15% by mass or less on the basis of the total amount of the composition.

## &lt;Physical Properties and Application&gt;

In the lubricating oil composition for a transmission of the present embodiment, it is preferred that a Brookfield viscosity (BF viscosity) at  $-40^{\circ}\text{C}$ ., a kinematic viscosity at  $40^{\circ}\text{C}$ ., a kinematic viscosity at  $100^{\circ}\text{C}$ ., and a viscosity index fall the following ranges, respectively. In the present embodiment, the BF viscosity is one as measured in conformity with ASTM D2983-09.

From the viewpoint of exhibiting the stable effects in a low-temperature region, the BF viscosity at  $-40^{\circ}\text{C}$  is preferably 30,000 mPa·s or less, more preferably 15,000 mPa·s or less, and still more preferably 7,500 mPa·s or less.

From the viewpoint of a balance between the gear properties and the cooling properties, the kinematic viscosity at  $40^{\circ}\text{C}$  is preferably 15 to 50 mm $^2$ /s, and more preferably 20 to 40 mm $^2$ /s.

From the viewpoint of a balance between the gear properties and the cooling properties, the kinematic viscosity at  $100^{\circ}\text{C}$  is preferably 3 to 15 mm $^2$ /s, and more preferably 4 to 10 mm $^2$ /s.

From the viewpoint of exhibiting the stable effects in a wide temperature region, the index viscosity is preferably 100 or more, more preferably 150 or more, and still more preferably 170 to 230.

In addition, in the lubricating oil composition for a transmission of the present embodiment, from the viewpoint of insulating properties, its volume resistivity is preferably  $1.0 \times 10^7 \Omega \cdot \text{m}$  or more, and more preferably  $2.5 \times 10^7 \Omega \cdot \text{m}$  or more. Although an upper limit of the volume resistivity of the lubricating oil composition for a transmission is not particularly limited, it is typically about  $1.0 \times 10^5 \Omega \cdot \text{m}$ .

For example, when the base oil as the component (A), the synthetic oil as the component (A-1), the viscosity index improver as the component (B), and the polyamide (C-1) and/or the polyol ester (C-2) are blended within the aforementioned suitable ranges, respectively, the volume resistivity can be made to fall within the aforementioned range.

In the present embodiment, the volume resistivity is one as measured at room temperature of  $25^{\circ}\text{C}$ . in conformity with the volume resistivity test of JIS C2101:1999.

In addition, in the lubricating oil composition for a transmission of the present embodiment, from the viewpoint of gear properties, its viscosity decrease in the shear stability test at  $100^{\circ}\text{C}$ . by the ultrasonic method (shear stability at  $100^{\circ}\text{C}$ .) is preferably 5.0% or less, more preferably 3.0% or less, and still more preferably 2.0% or less.

The viscosity decrease in the shear stability test is a value obtained by measuring the kinematic viscosity at  $100^{\circ}\text{C}$ . before the shear stability test and after the shear stability test in accordance with JIS K 2283:2000, followed by calculation according to the following equation (1). In addition, the shear stability test was performed based on the ultrasonic A method (JPI-5S-29) under a measurement condition for an ultrasonic irradiation time of 60 minutes at room temperature in an oil amount of 30 cc. An output voltage at which after irradiating 30 cc of a standard oil with ultrasonic waves for 10 minutes, the kinematic viscosity decrease at  $100^{\circ}\text{C}$ . reached 25% was defined as the output voltage of the ultrasonic waves in the shear stability test.

$$\text{Shear stability (\%)} = \frac{(\text{Kinematic viscosity before the test}) - (\text{Kinematic viscosity after the test})}{(\text{Kinematic viscosity before the test})} \times 100 \quad (1)$$

The lubricating oil composition for a transmission of the present embodiment can be used as a lubricating oil composition for a transmission of, for example, a gasoline car, a hybrid car, an electric car, or the like. In particular, because of excellent cooling properties and insulating properties, the lubricating oil composition for a transmission of the present embodiment can be suitably used as a lubricating oil composition for a transmission of a hybrid car or an electric car. More specifically, the lubricating oil composition for a transmission of the present embodiment can be suitably used as a lubricating oil composition for a combined use of transmission and motor cooling of a hybrid car or an electric car, or as a lubricating oil composition for a combined use of reduction gears and motor cooling.

## EXAMPLES

Next, the present invention is hereunder described in more detail by reference to the Examples, but it should be construed that the present invention is by no means limited by these Examples.

## 1. Preparation of Lubricating Oil Composition

A lubricating oil composition for a transmission of each of the Examples and Comparative Examples was prepared in a composition ratio shown in Table 1.

## 2. Measurement and Evaluation

With respect to the lubricating oil composition of each of the Examples and Comparative Examples, the following measurements and evaluations were performed. Results are shown in Table 1.

## 2-1. Kinematic Viscosity

The lubricating oil composition for a transmission was measured with respect to a kinematic viscosity at  $40^{\circ}\text{C}$ ., a kinematic viscosity at  $100^{\circ}\text{C}$ ., and a viscosity index in conformity with JIS K2283:2000.

## 2-2. Brookfield Viscosity (BF Viscosity)

The lubricating oil composition for a transmission was measured with respect to a BF viscosity at  $-40^{\circ}\text{C}$ . in conformity with ASTM D2983-09.

## 2-3. Gear Properties

## 2-3-1. FZG Gear Test

The test was performed under a condition at  $90^{\circ}\text{C}$ . and 1,450 rpm for 15 minutes in conformity with ASTM D5182-97 (2014), and a load stage at which scuffing was generated was measured.

## 2-3-2. Shear Stability

A kinematic viscosity at  $100^{\circ}\text{C}$ . before the shear stability test and after the shear stability test was measured in conformity with JIS K2283:2000, and a shear stability was calculated according to the following equation. In addition, the shear stability test was performed based on the ultrasonic

A method (JPI-5S-29) under a measurement condition for an ultrasonic irradiation time of 60 minutes at room temperature in an oil amount of 30 cc. An output voltage at which after irradiating 30 cc of a standard oil with ultrasonic waves for 10 minutes, the kinematic viscosity decrease at  $100^{\circ}\text{C}$ . reached 25% was defined as the output voltage of the ultrasonic waves in the shear stability test.

$$\text{Shear stability (\%)} = \frac{(\text{Kinematic viscosity before the test}) - (\text{Kinematic viscosity after the test})}{(\text{Kinematic viscosity before the test})} \times 100$$

## 2-4. Clutch Properties

An engagement test in which an inertial plate rotating at 3,600 rpm was made stationary due to friction between a

friction plate (FZ127-24-Y1) and a steel plate (FZ132-8-Y1) by using an SAE No. 2 tester (friction properties tester) was performed in conformity with JASO M348-95; and a friction coefficient  $\mu_{1800}$  at a rotation rate of 1,800 rpm on the way of being made stationary and a friction coefficient  $\lambda_{200}$  at a rotation rate of 200 rpm just before stop were measured, and  $\mu_{200}/\mu_{1800}$  was calculated. A surface pressure was set to 1 MPa, and an oil temperature was set to 100°C.

It may be said that as the  $\mu_{200}/\mu_{1800}$  is small, the shift shock at the time of clutch connection is suppressed, so that the clutch properties are excellent.

#### 2-5. Insulating Properties (Volume Resistivity)

A volume resistivity (S·m) of the lubricating oil composition for a transmission was measured at room temperature of 25°C. in conformity with the volume resistivity test of JIS C2101:1999.

#### 2-6: Cooling Properties

A silver rod heated at 200°C. was put into a sample oil heated at 80°C. in conformity with the "cooling properties test method: A method" as prescribed in JIS K2242:2012; a cooling curve was prepared from a temperature change on the silver rod surface, and a cooling rate (deg/s) of the cooling curve at 200°C. was calculated.

TABLE 1

|                              |                                                                                                        | Exam-<br>ple 1                                            | Exam-<br>ple 2    | Exam-<br>ple 3    | Compar-<br>ative<br>Example 1 | Compar-<br>ative<br>Example 2 | Compar-<br>ative<br>Example 3 | Compar-<br>ative<br>Example 4 | Compar-<br>ative<br>Example 5 |
|------------------------------|--------------------------------------------------------------------------------------------------------|-----------------------------------------------------------|-------------------|-------------------|-------------------------------|-------------------------------|-------------------------------|-------------------------------|-------------------------------|
| Compo-<br>sition<br>(mass %) | (A) Base oil                                                                                           | (A-1) Synthetic oil<br>Other synthetic oil<br>Mineral oil | 3<br>6.6<br>71    | 3<br>6.6<br>71    | 3<br>6.6<br>71                | 0<br>0<br>79                  | 0<br>0<br>71                  | 0<br>0<br>83                  | 74<br>14<br>0                 |
|                              | (B) Viscosity index improver                                                                           | 7                                                         | 7                 | 7                 | 11                            | 8                             | 11                            | 0                             | 0                             |
|                              | Other viscosity index improver                                                                         | 0                                                         | 0                 | 0                 | 0                             | 0.6                           | 0                             | 4.5                           | 0                             |
|                              | (C-1) Polyamide                                                                                        | 0.1                                                       | 0.1               | 0                 | 0                             | 0                             | 0                             | 0.1                           | 0                             |
|                              | (C-2) Polyol ester                                                                                     | 0.1                                                       | 0                 | 0.1               | 0                             | 0                             | 0                             | 0.1                           | 0                             |
| Properties                   | Additives (friction modifier, antioxidant, dispersant, pour-point depressant, antifoaming agent, etc.) | Balance                                                   | Balance           | Balance           | Balance                       | Balance                       | Balance                       | Balance                       | Balance                       |
|                              | Kinematic viscosity at 40°C. (mm <sup>2</sup> /s)                                                      | 27                                                        | 27                | 27                | 27                            | 30                            | 33                            | 35                            | 16.5                          |
|                              | Kinematic viscosity at 100°C. (mm <sup>2</sup> /s)                                                     | 6.2                                                       | 6.2               | 6.2               | 6.2                           | 7.2                           | 7.2                           | 7.2                           | 4.3                           |
|                              | Viscosity index                                                                                        | 192                                                       | 192               | 192               | 192                           | 218                           | 192                           | 180                           | 185                           |
|                              | BF viscosity (mPa · s)                                                                                 | 6000                                                      | 6000              | 6000              | 6000                          | 6800                          | 6800                          | 18000                         | 3000                          |
| Evaluation                   | Gear properties                                                                                        | FZG gear test<br>Shear stability (%)                      | 11<br>1.5%        | 11<br>1.5%        | 11<br>1.5%                    | 11<br>5.8%                    | 11<br>1.5%                    | 11<br>14.8%                   | 10<br>1.5%                    |
|                              | Clutch properties                                                                                      | $\mu_{200}/\mu_{1800}$                                    | 0.992             | 1.000             | 1.000                         | 1.008                         | 1.008                         | 1.008                         | 0.992                         |
|                              | Electric insulating properties                                                                         | Volume resistivity<br>( $\Omega \cdot m$ )                | $3.5 \times 10^7$ | $3.5 \times 10^7$ | $3.5 \times 10^7$             | $3.5 \times 10^7$             | $3.5 \times 10^7$             | $3.5 \times 10^7$             | $3.5 \times 10^7$             |
|                              | Cooling properties (deg/s)                                                                             |                                                           | 7.5               | 7.5               | 7.5                           | 7.0                           | 7.0                           | 7.0                           | 8.0                           |

The materials of Table 1 are as follows.

(A-1) Synthetic oil: Poly- $\alpha$ -olefin (polydecene, kinematic viscosity at 40°C.: 5.1 mm<sup>2</sup>/s, kinematic viscosity at 100°C.: 1.8 mm<sup>2</sup>/s, viscosity index: 128)

Other synthetic oil: Kinematic viscosity at 40°C.: 1,240 mm<sup>2</sup>/s, kinematic viscosity at 100°C.: 100 mm<sup>2</sup>/s

Mineral oil: Kinematic viscosity at 40°C.: 9.9 mm<sup>2</sup>/s, kinematic viscosity at 100°C.: 2.7 mm<sup>2</sup>/s

(B) Viscosity index improver (polymethyl methacrylate, Mw: 30,000)

Other viscosity index improver (polymethyl methacrylate, Mw: 100,000)

(C-1) Polyamide: A reaction product between stearic acid and aliphatic polyamine

(C-2) Polyol ester: A mixture of oleic acid monoglyceride and oleic acid diglyceride

As is clear from the results of Table 1, the lubricating oil compositions for a transmission of Examples 1 to 3 could simultaneously satisfy the gear properties, the clutch properties, the cooling properties, and the insulating properties.

In addition, the lubricating oil compositions for a transmission of Examples 1 to 3 were able to suppress an increase of the BF viscosity at -40°C., so that the stable effects could be expected even in a low-temperature region.

On the other hand, the lubricating oil compositions for a transmission of Comparative Examples 1 to 5 are ones not containing at least one of the synthetic oil (A-1) having a kinematic viscosity at 100°C. of 1.0 to 10.0 mm<sup>2</sup>/s, the viscosity index improver (B) having a mass average molecular weight of 10,000 to 50,000, and the polyamide (C-1) and/or the polyol ester (C-2). For that reason, the lubricating oil compositions for a transmission of Comparative Examples 1 to 5 could not simultaneously satisfy the gear properties, the clutch properties, the cooling properties, and the insulating properties.

#### INDUSTRIAL APPLICABILITY

The lubricating oil composition for a transmission of the present embodiment is useful from the standpoint that it is able to simultaneously satisfy gear properties (e.g., seizure resistance or shear stability under a high load), clutch

properties (e.g., suppression of shift shock at the time of clutch connection), cooling properties, and electric insulating properties.

The invention claimed is:

1. A lubricating oil composition, comprising:
  - (A) a base oil comprising (A-1) a synthetic oil having a kinematic viscosity at 100°C. of 1.0 to 10.0 mm<sup>2</sup>/s;
  - (B) a viscosity index improver having a mass average molecular weight of 10,000 to 50,000;
  - (C-1) a polyamide, which is a reaction product between a polyamine compound and a carboxylic acid compound, wherein the carboxylic acid compound is a monovalent fatty acid having a carbon number from 8 to 24; and
  - (C-2) a polyol ester which is a partial ester of a polyol and a fatty acid having 12 to 24 carbon atoms, wherein a total amount of the component (C-1) and the component (C-2) is from 0.01 to 5.0% by mass on the basis of a total amount of the composition.
2. The composition of claim 1, wherein the component (A-1) is a poly- $\alpha$ -olefin, a hydrogenated product of a poly- $\alpha$ -olefin, or both.

**11**

3. The composition of claim 1, wherein the component (A-1) is present in an amount from 1.0 to 10.0% by mass on the basis of a total amount of the composition.

4. The composition of claim 1, wherein the component (B) is a poly(meth)acrylate.

5. The composition of claim 1, wherein the component (B) is present in an amount from 1.0 to 20.0% by mass on the basis of a total amount of the composition.

6. The composition of claim 1, having a kinematic viscosity at 100° C. of 3 to 15 mm<sup>2</sup>/s.

7. The composition of claim 1, having a viscosity index of 100 or more.

8. The composition of claim 1, having a volume resistivity of 1.0×10<sup>7</sup> Mu or more.

9. The composition of claim 1, having a Brookfield viscosity at -40° C. of 30,000 mPas or less.

10. The composition of claim 1, wherein the polyamine compound is an aliphatic polyamine having a total carbon number of 6 to 30, and

wherein the carbon number of the hydrocarbon group of the carboxylic acid is from 12 to 24.

11. The composition of claim 10, wherein the aliphatic polyamine has a total carbon number of 16 to 24, and wherein the carbon number of the hydrocarbon group of the carboxylic acid compound is from 18 to 22.

12. The composition of claim 1, wherein the base oil further comprises a mineral oil having a kinematic viscosity at 100° C. of 1.5 to 6 mm<sup>2</sup>/s,

wherein the composition comprises from 60.0 to 90.0% by mass of the mineral oil on the basis of a total amount of the composition and from 1.0 to 10.0% by mass of the synthetic oil (A-1) on the basis of a total amount of the composition.

**12**

13. The composition of claim 11, wherein the component (B) is present in an amount from 3.0 to 15.0% by mass on the basis of a total amount of the composition.

14. The composition of claim 1, further comprising: a friction modifier which is neither the polyamide (C-1) nor the polyol ester (C-2), and a pour point depressant which is neither the polyamide (C-1) nor the polyol ester (C-2).

15. The composition of claim 1, wherein the polyol of the polyol ester (C-2) comprises trimethylolethane, ditrimethylolethane, trimethylolpropane, ditrimethylolpropane, glycerin, pentaerythritol, dipentaerythritol, tripentaerythritol, or sorbitol, and

wherein the carboxylic acid of the polyol ester (C-2) comprises stearic acid or oleic acid.

16. The composition of claim 1, wherein the base oil further comprises a mineral oil having a kinematic viscosity at 100° C. of 1.5 to 6 mm<sup>2</sup>/s, and

wherein the composition comprises from 60.0 to 90.0% by mass of the mineral oil on the basis of a total amount of the composition and from 2.0 to 5.0% by mass of the synthetic oil (A-1) on the basis of a total amount of the composition,

with a balance comprising further synthetic oil.

17. The composition of claim 1, having a kinematic viscosity at 100° C. of 3 to 15 mm<sup>2</sup>/s, and having a viscosity index of 150 or more.

18. The composition of claim 1, wherein the total amount of the component (C-1) and the component (C-2) is from 0.01 to 1.0% by mass on the basis of a total amount of the composition.

\* \* \* \* \*